

# UNITED STATES PATENT OFFICE.

HARRY G. AKERS, OF TORONTO, ONTARIO, CANADA.

## PROCESS OF PRODUCING BARIUM AND STRONTIUM OXIDS.

1,113,178.

Specification of Letters Patent.

Patented Oct. 13, 1914.

No Drawing.

Application filed May 8, 1913. Serial No. 766,410.

To all whom it may concern:

Be it known that I, HARRY G. AKERS, a citizen of Canada, and subject of the King of Great Britain, residing at Toronto, in the Province of Ontario and Dominion of Canada, have invented certain new and useful Improvements in Processes of Producing Barium and Strontium Oxids; and I do hereby declare the following to be a full, clear, and exact description of the invention, such as will enable others skilled in the art to which it appertains to make and use the same.

This invention relates to the production of barium and strontium oxids from their carbonates, and has for its purpose to provide a process which will accomplish these objects in a manner more efficient and expeditious than those heretofore proposed.

With these and other objects in view the invention consists in the novel steps and combinations of steps constituting my process, all as are more fully hereinafter disclosed and particularly pointed out in the claims.

As is well known, barium or strontium carbonates which have been employed in the refining of molasses and therefore are more or less contaminated with lime, silica, organic substances, etc., are difficult to fuse, and do not even melt at 1200° C. or 1300° C., the exact temperature depending upon the amount and character of the impurities present. I have discovered, however, that these impure carbonates can be readily melted at approximately 1200° C. by adding small quantities of fluxes, such as fluor-spar, soda ash, borax, etc., the best quantity being readily determined by simple and well known tests, and depending upon the character and quantity of the impurities in the carbonates. I have further discovered that after the said carbonates, whether pure or not, have been melted they may be readily changed into oxids almost to completion at temperatures approximating to 1200° C. provided the partial pressure of the carbon dioxid liberated by the reaction be kept below that of the atmosphere and sufficient carbon be present. In some cases I have found a carbon lining for portions of the furnace to yield good results, as it tends to assist in changing the carbonates into oxids, and it is comparatively inexpensive to renew.

In carrying out my process the barium

or strontium carbonates according to the nature of the impurities present may be with or without an admixed reducing agent, depending upon the subsequent treatment 60 said carbonates are to receive, fed into a suitable furnace such, for example, as a rotary cement kiln. The charge mixed with a flux may be conveniently in the form of a sludge, in which form it usually comes 65 from the carbonating tanks, and can be dried in the stack end of the furnace by means of the exit gases. This charge may then be melted in the body of the furnace and admixed with a reducing agent as it is 70 fed along, if no such agent be already present, and finally delivered into a suitable receptacle in a molten condition.

By so proportioning the carbon or other reducing agent as to compel a large proportion of the carbon monoxid instead of carbon dioxid to be given off, the exit gases will consist largely of nitrogen and carbon monoxid, CO mixed with a less quantity of carbon dioxid, CO<sub>2</sub>, the partial pressure of 80 the latter will be low and the full value of said gases may be employed to assist the heating and reduction of the charge. In 75 other words, by the simple expedients of adding a flux to these carbonates to allow 85 them to fuse at approximately 1200° C. and mixing them with a carbonaceous substance, I accomplish the most desirable results of attaining a lower melting point for 90 said carbonates, which allows a better contact between the carbonate and the reducing agent and consequently allows the reduction to proceed readily at comparatively 95 low temperatures. Further, the lowering of the said partial pressure greatly facilitates 100 the reduction of the carbonates and enables me to accomplish the reduction to almost completion at temperatures approximating 1200° C. as above stated, a result which would not be possible by the old methods, 105 while at the same time the larger quantity of carbon monoxid produced, enables me to get a higher fuel value from the exit 110 gases to aid in the reduction.

While the charge is in its molten condition it is sometimes desirable to further refine it by introducing a reducing agent by means of a nozzle delivering compressed air charged with said agent in a finely divided condition, or said agent may be blown 110 through the molten material. These latter expedients will be also useful when the

reducing agent has not been initially mixed with the charge as above referred to or was admixed therewith in an insufficient quantity, or has been burnt out by the gases produced in the previous stages of the process.

The advantages of my process will be apparent when one considers the economy due to the drying and preheating of the crude carbonates which are usually in the form of a sludge, the continuity of the process, the cheapness of the equipment necessary for carrying it out, the lower temperature and less heat required for the separation, and the overcoming of the present necessity for heating the charge through the walls of a crucible or other vessel in which these crude carbonates are now usually treated.

It is obvious that those skilled in the art may vary the details of my process without departing from the spirit of my invention, and therefore I do not wish to be limited to the above disclosure, except as may be required by the claims.

What I claim is:—

25. 1. The continuous process of producing barium or strontium oxids from their crude carbonates which consists in mixing the carbonate with a flux to lower its melting point; adding a reducing agent to the charge; melting the charge at a temperature of approximately 1200° C.; igniting the evolved gases to heat the charge and to preheat the incoming charge; and maintaining a reducing atmosphere in the reacting vessel containing said charge, substantially as described.

2. The continuous process of producing barium or strontium oxids from their crude carbonates which consists in mixing the carbonates with a flux to lower the melting point; adding a reducing agent to the charge; melting the charge at a temperature of approximately 1200° C.; igniting the evolved gases to heat the charge and to preheat the incoming charge; maintaining a reducing atmosphere in the reacting vessel

containing said charge; and causing the gases produced by the combustion of the fuel employed in heating the furnace to dilute and thereby lower the partial pressure 50 of any evolved carbon dioxid from said charge, substantially as described.

3. The continuous process of producing barium or strontium oxids from their crude carbonates which consists in mixing the carbonates with a flux to lower the melting point; adding a reducing agent to the charge; melting the charge at a temperature of approximately 1200° C.; refining the mass by again adding a reducing agent; 60 causing the gases produced by the combustion of the fuel employed in heating the furnace to dilute any liberated carbon dioxid and thereby reduce its partial pressure; igniting the evolved gases to heat the charge 65 and to preheat the incoming charge; and maintaining a reducing atmosphere in the reacting vessel containing said charge, substantially as described.

4. The continuous process of producing 70 barium or strontium oxids from their crude carbonates in the form of a sludge which consists in mixing the carbonates with a flux to lower the melting point; adding a reducing agent to the charge; melting the charge 75 at a temperature of approximately 1200° C. in a carbon lined furnace; igniting the evolved gases to heat the charge and to preheat the incoming charge; maintaining a reducing atmosphere in the reacting vessel 80 containing said charge; and causing the gases produced by the combustion of the fuel employed in heating the furnace to dilute and thereby lower the partial pressure of any evolved carbon dioxid from said 85 charge, substantially as described.

In testimony whereof I affix my signature, in presence of two witnesses.

HARRY G. AKERS.

Witnesses:

G. O. KINGSTON,  
J. JORDAN.